# EUROPEAN PATENT SPECIFICATION

(11) **EP 0 121 029 B1**
(45) Date of publication and mention of the grant of the patent: **08.04.1987**
(21) Application number: 83420059.4
(22) Date of filing: 30.03.1983
(51) Int. Cl.: F27D 1/16

(54) **A method for the gunning of basic gunning refractories**
Verfahren zum Spritzen von basischen feuerfesten Stoffen
Méthode de projection de réfractaires basiques

(43) Date of publication of application: 10.10.1984
(73) Proprietor: AIKOH CO. LTD., Tokyo (JP)
(72) Inventor: Takashima, Masaru, Tokyo (JP)
(74) Representative: Maureau, Pierre

## Description

This invention relates to a gunning method in which basic gunning refractories are suitably coated or filled to construction, vessel and apparatus for which a refractory property is required.

These days unshaped refractories are in quick spread due to their effectiveness for the improvement of working efficiency and there are introduced various working methods utilizing vibration, centrifugal force, pressure force, injection, gunning, etc. as well as pouring, and feeding under pressure. However, in carrying out the working methods they have problems peculiar to each thereof, and particulary for the gunning method there is left room of improvement in obtaining an even adhesion layer with good yield, owing to rebound loss or droop.

In these circumstances the inventor of this invention has noticed that in gunning the basic refratories a dry gunning by nozzle mixing in which solid and liquid are mixed at the nozzle portion is superior in obtaining the adhesion layers of excellent refractory and anti-corrosive properties, in cooperation with the adoption of basic refractories, to a wet gunning of using refractory slurry, and as a result of having studied the adaptation of gunning refractories and gunning conditions he has been able to obtain an effective knowledge thereby to improve said problems concerning the coating or filling irrespective of cold gunning or hot gunning and to make the present invention in which the present gunning method can be conveniently applied.

According to the present invention it is possible to form a strong, refractory layer at any place where refractory coating or filling is needed, irrespective of plane, curved surface, concave portion, void portion, and the inner surface or the outer surface of tubular body, not to speak of melting furnaces such as blast furnace, converter, electric furnace and reverberatory furnace, vessels for molten metal such as ladle and tundish, vessels for treating molten metals used in Rheinetahl-Hereus process and Dortmund Huttenunion process, various industrial, heating furnaces, various accessories and accessory positions of all these furnaces and vessels, and appliances and apparatuses used in accompanying working. It is also possible to resolve the problem such as rebound loss or droop.

The object of the invention is to provide a method for the gunning of a basic gunning refractory in which there is carried out a cold or hot gunning coating or filling, by a nozzle mixing- method, of a gunning refractory containing a basic refractory as aggregate , not more than 5% by weight of at least one of organic fibrous materials and inorganic fibrous materials, and as binder, at least one of phosphates and silicates, wherein the gunning refractory is fed to the nozzle portion under air pressures in the range of 1-10 kg/cm² (0.981-9,81 bars), said gunning refractory is then discharged while being mixed at said nozzle portion with 5-25% by weight of water having teh pressure in the range 0.5-5 Kg/cm² (0.49―4,905 bars) and while being accompanied by a rotary motion, the gunning order at the start of discharging takes first air and water simultaneously and then the gunning refractories, and the distance between the nozzle end and the gunning surface is in the range 0.15 to 1.00 m while the gunning width is less than 1.00 m.

The reason of using basic refractories as aggregate of the gunning refractory in effecting the present invention is that not only they are excellent in both refractoriness and load softening point but particularly they exhibit an excellent melting-down resistancy against high temperature under the co-existence with basic slag, and as the basic refratories there can be used more than one selected from among magnesia refractories such as magnesia clinker, dolomite, clinker, peridottite, chrome magnesia and magnesia spinel, and lime refractories such as sintered calcia, larnite and quick lime.

Organic and inorganic fibrous materials enhance the porosity of the gunning, coating layer, have smaller bulk specific density and improve the spalling resistancy of said coating layer so that at least one of both of them is mixed up to 5% by weight. Even with the addition thereof by more than 5% by weight any improved effect is not noticed but to the contrary it degrades the mechanical strength (compressive strength). As such fibrous materials the following can be mentioned.

That is, there can be used animal and vegetation fibers such as pulp, beaten paper, cotton, wool, silk and synthetic fibers, as organic fibrous materials, and heat resistant fibers such as asbestos, rock wool, slag wool, ceramic fibers and carbon fibers, as inorganic fibrous materials.

Phosphates and silicates used as binder are known as binder for refractory aggregate, and there can be used more than one selected from among alkali metal salts, alkali earth metal salts and aluminium salts or orthophosphoric acid, polyphosphoric acid, methaphosphoric acid and ultraphosphoric acid with regard to phosphates, and from among alkali metals of silicic acid with regard to silicates.

Further, it is possible to selectively add, to the gunning refractory, a carbonaceous material or inorganic or organic viscosity-increasing agent besides the above materials, as necessary.

The gunning refractory is fed to the nozzle portion under air pressures from 1 to 10 Kg/cm2 (0.981-9.81 bars) and discharged while being mixed with water under pressures in the range 0.5-5 Kg/cm² (0.49―4.905 bars) and while being accompanied by a rotary motion in said nozzle portion. The reason why the gunning refractory is fed under air pressures in the range 1 to 10 Kg/ cm² (0.981-9.81 bars) is that it is possible to optionally take the mode of discharging ranging from gunning and beating to a condition like flowing-out, and with 1 Kg/cm² (0.981 bar) the air pressure is not sufficient while 10 Kg/cm² (9.81 bars) air pressure is too great whereby neither of the cases can achieve the object of the present invention. To prevent the nozzle from blocking, the gunning order at the time of starting the discharge is brought in such a way that the air and the water are discharged simultaneously and then the gunning refractory is discharged.

The opening for supplying water in said nozzle portion can be provided by single or plurarity in optional position and mode in the nozzle portion to effect a nozzle mixing. The amount of supplying water is from 5 to 25% by weight to the gunning refractory, less than 5% by weight of water is too little to make a complete mixing and to have a sufficient adhesion strength while more than 25% by weight is too great so as to flow the the gunning refractory away whereby neither of the cases forms a sufficient coating layer.

If is one of the important constitutional features of the invention to discharge said mixture with a rotary motion, and as a method of making the rotary motion it is effective, for example, to provide the opening for feeding the gunning refractory to the nozzle portion, tangentially to the cross section of said nozzle, and it is also preferably to use a plate like guide plate along the rotational direction within the nozzle portion, by alone or in co-use with said opening. Further, it is effective, as an auxiliary means for imparting the rotary motion, to arrange the opening or openings for supplying water in the tangential direction along the rotational direction of said gunning refractory. In any case it is capable of optionally selecting the rotational direction of said gunning refractory in the designing process of nozzle.

As the gunning conditions regarding the nozzle operation, the distance from the nozzle to the gunning surface is in the range of 0.15 to 1.00 m, and with less than 0.15 m distance the gunning refractory is greatly lost by rebound while if the distance exceeds 1.00 m the discharging energy is lowered, so that any of such cases does not form a preferable coating layer. Furthermore, the reason why the gunning width of the gunning refractory in the gunning surface is less than 1.00 m is that it is related to said distance between the nozzle and the gunning surface, and in case the gunning width is more than 1.00 m it is no longer possible to obtain a useful coating layer. The adjustable range of more suitable gunning width is from 0.05 to 1.00 m.

The angle to the gunning surface of the nozzle may be as near right angle (vertical) as possible, but practically an angle of more than 45 degrees will suffice since it hardly causes rebound and it is almost same as in right angle. Said angle of the nozzle can be changed by turning the nozzle arm or curving or bending the tip portion of the nozzle. As the operating apparatus it will be proper to use an automatic operation apparatus provided with various functions such as travelling, moving sidewise and vertically and turning.

Referring to the temperaturs of the gunning surface, the temperature range wherein the present invention can be effected is 0-1,000°C whichever in cold gunning or hot gunning. If it is below 0°C, the gunning freezes and if it exceeds 1,000°C the water content quickly evaporates so that in both cases it becomes difficult to gun the refractory.

The discharge amount from the nozzle is in the range 5-25 Kg/min, and with less the 5 Kg/min or with 25 kg/min the discharge amount is too little or too much whereby in both the cases gunning becomes impossible.

The nozzle to the gunning surface can move in one of the optional directions accompanied by reciprocal movement and spiral movement. Naturally a reverse case may occur to the case in which the moving direction of said nozzle accords with the rotational movement direction of said gunning refractory, but in any case the object of the present invention is achievable. The moving speed of the nozzle to the gunning surface is 30 m/min during the gunning, and to be speedier than 30 m/min is too fast so that the adhesion of the gunning refractory becomes incomplete due to the rebounding of the refractory from the gunning surface.

Whether to move the nozzle during the gunning by hand or automatically does not reversely affect the function and effect of the invention if the variety of the above conditions are satisfied, but from the safety point of view of working it would be better to use an automated machine.

Now referring to the nozzle employed in the method of this application, it is provided at the peripheral edge of the tip air injection ports which form an air curtain at the tip of the gunning direction, so as to prevent the gunning refractory from scattering. Further, to prevent the nozzle from blocking, gunning is carried out with a nozzle, at least part of which is provided with a rotational machanism.

The following is an example in which the present invention was carried out for lining a surface of refractory bricks of a tundish for continuous steel casting.

A gunning was effected in such a manner that a gunning refractory consisting of a mixture of 86% by weight of magnesia clinker, 4% by weight of rock wool, 3% by weight of waste cotton, 4% by weight of sodium primary phosphate and 3% by weight of sodium methasilicate, was fed to the nozzle portion under an air pressure of 5.3 Kg/cm² (5.199 bars) from the tangential direction to the cross section of the nozzle, while being supplied 11 % by weight of water of the gunning refractory from the circumferential apertures in said nozzle portion. Retaining the distance between the nozzle and the gunning surface with 0.4 m and the gunning angle with approximately 90° the nozzle was moved spirally along the inner circumference at the speed of 1 m/min. Moreover, the temperature at the gunning surface just before the starting of the gunning was 500°C, when a coating layer of 0.2 m adhesion width was obtained at a discharge rate of 15Kg/min. Under such conditions the gunning refractory was discharged while being mixed with water and being accompanied by a rotary motion, the gunning refractory was adhered uniformly and smoothly to the gunning surface since being subject to a rectifying control by an intermediated squeezing portion, the rebound loss was only 10% though it was 30-40% according to conventional method, and droop was not noticed thereby improving the conventional problems.

An average thickness of 0.015 m was made to the coating layer of the tundish and the tundish was preheated at 1,000°C for 30 minutes just before its operation, but craking or any other phenomena occurred, the coating layer could stand the use of continuous-continuous castings of 5 charges of 200 ton steel melt, and the remaining minimum thickness of the coating layer was still 0.01 m at the finish of the casting so that a satisfactory result could be obtained.

## Claims

1. A method for the gunning of a basic gunning refractory in which there is carried out a cold or hot gunning coating or filling, by a nozzle mixing method, of a gunning refractory containing a basic refractory as aggragate, not more than 5% by weight of at least one or organic fibrous materials and inorganic fibrous materials, and as binder, at least one of phosphates and silicates, wherein the gunning refractory is fed to the nozzle portion under air pressures in the range 1-10 Kg/ cm² (0.981-9.81 bars) said gunning refractory is then discharged while being mixed at said nozzle portion with 5-25% by weight of water having the pressure in the range' 0.5-5 kg/cm² (0.49―4,905 bars) and while being accompanied by a rotary motion, the gunning order at the start of discharging takes first air and water simultaneously and then the gunning refractory, and the distance between the nozzle end and the gunning surface is in the range 0.15 to 1.00 m while the gunning width is less than 1.00 m.

2. A method for the gunning of a basic gunning refractory as described in Claim 1 wherein the temperature of the gunning surface is in the range 0-1,000°C in cold or hot gunning.

3. A method for the gunning of a basic gunning refractory as described in any of Claims 1 or 2 wherein the gunning refractory is imparted with a rotational motion in a predetermined, optional direction in the nozzle portion.

4. A method for the gunning of a basic gunning refractory as described in any of Claims 1 to 3, wherein the discharged amount from th nozzle is in the range 5-25 Kg/min.

5. A method for the gunning of a basic gunning refractory as described in any of Claims 1 to 4 wherein the gunning width is in the range 0.05-1.00 m.

6. A method for the gunning of a basic gunning refractory as described in any of Claims 1 to 5 wherein the nozzle is moved in any optional one direction being accompanied by a reciprocating movement of a spiral movement.

7. A method for the gunning of a basic gunning refractory as described in any of Claims 1 to 6 wherein the travelling speed of the nozzle is slower than 30 m/min.

8. A method for the gunning of a basic gunning refractory as described in any of Claims 1 to 7, wherein there is used a nozzle provided with air injection apertures which form an air curtain in the discharging direction.

9. A method for the gunning of a basic gunning refractory as described in any of Claims 1 to 8 wherein the gunning is carried out by rotating at least a part of the nozzle.

## Patentansprüche

1. Verfahren zum Spritzen von basischen feuerfesten Spritzmaterialien, dadurch gekennzeichnet, daß kalt oder heiß mittels eines Düsen-Mischverfahrens eine Deckschicht oder ein Füller aus einem feuerfesten Spritzmaterial aufgetragen wird, welches ein basisches feuerfestes Material als Zuschlagstoff enthält, nicht mehr als 5 Gewichtsprozente wenigstens entweder eines organischen Fasermaterials oder eines anorganischen Fasermaterials, sowie als Binder wenigstens entweder Phosphate oder Silikate, wobei das feuerfeste Spritzmaterial mittels eines Luftdruckes im Bereich von 1-10 kg/cm² (0,981-9,81 bar) dem Düsenabschnitt zugeführt und das feuerfeste Spritzmaterial sodann ausgespritzt wird, während es in diesem Düsenabschnitt mit 5-25 Gewischtsprozenten Wasser unter einem Druck im Bereich von 0,5-5 kg/cm² (0,49―4,905 bar) gemischt und dabei gleichzeitig einer Rotationsbewegung unterzogen wird, daß in der Spritzfolge zu Beginn des Ausspritzens zunächst Luft und Wasser gleichseitig und dann das feuerfeste Spritzmaterial mitgenommen wird, und daß der Abstand zwischen dem Düsenende und der Spritzoberfläche 'im Bereich von 0,15-1,00 m liegt, während die Spritzweite geringer als 1 m ist.

2. Verfahren zum Spritzen eines basischen feuerfesten Spritzmaterials nach Anspruch 1, dadurch gekennzeichnet, daß 'die Temperatur der Spritzoberfläche im Bereich von 0-1 000°C beim Kalt- oder Heißspritzen ist.

3. Verfahren zum Spritzen eines basischen feuerfesten Spritzmaterials nach Anspruch 1 oder 2, dadurch gekennzeichnet, daß das feuerfeste Spritzmaterial im Düsenabschnitt einer Rotationbewegung in einer vorbestimten und erwünschten Richtung unterwofen wird.

4. Verfharen zum Spritzen eines basischen feuerfesten Spritzmaterials nach einem der Ansprüche 1 bis 3, dadurch gekennzeichnet, daß die von der Düse ausgespritzte Menge im Bereich von 5-25 kg/min liegt.

5. Verfharen zum Spritzen eines basischen feuerfesten Spritzmaterials nach einem der Ansprüche 1 bis 4, dadurch gekennzeichnet, daß die Spritzweite im Bereich von 0,05-1 m liegt.

6. Verfharen zum Spritzen eines basischen feuerfesten Spritzmaterials nach einem der Ansprüche 1 bis 5, dadurch gekennzeichnet, daß die Düse jeweils wahlweise in einer Richtung bewegt wird, wobei diese Bewegung durch eine hin- und hergehende Bewegung einer Spiralbewegung begelietet wird.

7. Verfharen zum Spritzen eines basischen feuerfesten Spritzmaterials nach einem der Ansprüche 1 bis 6, dadurch gekennzeichnet, daß die Bewegungsgeschwindigkeit der Düse kleiner als 30 m/min. ist.

8. Verfharen zum Spritzen eines basischen feuerfesten Spritzmaterials nach einem der Ansprüche 1 bis 7, dadurch gekennzeichnet, daß eine mit Luftblaseöffnungen versehene Düse verwendet wird, welche irr Ausspritzrichtung einen Luftvorhang erzeugt.

9. Verfharen zum Spritzen eines basischen feuerfesten Spritzmaterials nach einem der Ansprüche 1 bis 8, dadurch gekennzeichnet, daß das Spritzen unter Rotieren wenigstens eines Teils der Düse ausgeführt wird.

## Revendications

1. Procédé de projection d'un produit réfractaire basique de projection selon lequel on effectue un revêtement ou un remplissage, par projection à froid ou à chaud, par un procédé de mélange dans la buse d'un réfrataire de projection renfermant comme agrégat un réfractaire basique, au maximum 5% en poids d'au moins un matériau choisi parmi les matériaux fibreux organiques et les matériaux fibreux inorganiques et, comme liant, au moins un produit choisi parmi les phosphates et silicates, dans lequel le réfractaire de projection est amené à la partie buse sous des pressions d'air se situant entre 1 et 10 Kg/cm² (0,981-9,81 bars), ledit réfractaire de projection étant alors évacué tout en étant mélangé dans ladite partie buse avec 5 à 25% en poids d'eau sous une pression de 0,5 à 5 Kg/cm² (0,49―4,905 bars), ceci étant accompagné d'un mouvement rotatif, la projection au démarrage de la projection, commençant d'abord et simultanément par l'air et par l'eau, puis les réfractairs de projection, et la distance entre l'extrémité de la buse et la surface de projection se situant entre 0,15 et 1,00 m tandis que la largeur de projection est inférieure à 1,00 m.

2. Procédé de projection d'un produit réfractaire basique selon la revendication 1, dans lequel la température de la surface de projection se situe entre 0 et 1.000°C, en projection à froid ou à chaud.

3. Procédé de projection d'un produit réfractaire basique selon la revendication 1 et la revendication 2, dans lequel le réfractaire de projection est amené avec un mouvement de rotation dans un sens optionnel et prédéterminé dans la partie buse.

4. Procédé de projection d'un produit réfractaire basique selon l'une des revendications 1 à 3, dans lequel la quantité qui sort de la buse se situe entre 5 et 25 Kg/min.

5. Procédé de projection d'un produit réfractaire basique selon l'une des revendications 1 à 4, dans lequel la largeur de projection se situe entre 0,05 et 1,00 m.

6. Procédé de projection d'un produit réfractaire basique selon l'une des revendications 1 à 5, dans lequel la buse est déplacée , optionnellement, dans un sens, ceci étant accompagné d'un déplacement réciproque hélicoïdal.

7. Procédé de projection d'un produit réfractaire basique selon l'une des revendications 1 à 6, dans lequel la vitesse de la buse est inférieure à 30 m/ min.

8. Procédé de projection d'un produit réfractaire basique selon l'une des revendications 1 à 7, dans lequel on utilise une buse équippée d'ouvertures pour injection de l'air, qui forment un rideau d'air dans la direction d'écoulement.

9. Procédé de projection d'un produit réfractaire basique selon l'une des revendications 1 à 8, dans lequel la projection est effectuée en faisant tourner au moins une partie de la buse.
